

## UNITED STATES PATENT OFFICE.

BYRAJJI D. SAKLATWALLA, OF CRAFTON, PENNSYLVANIA.

## ALLOY STEEL.

No Drawing.

Application filed July 7, 1923. Serial No. 850,157.

The present invention relates to manufacture of alloy steels, and more particularly to the reduction of the alloying elements directly from their ores, and the production 5 of the respective alloy steels, without the introduction of excess carbon in the finished steel.

In the manufacture of alloy steels, under the practice heretofore prevalent, the alloying elements, in the already reduced metallic state, mostly in the form of a ferro-alloy, are added to a molten bath of steel. For example, to obtain the respective steels thereof, ferro-manganese, ferro-chromium, 15 ferro-titanium, ferro-tungsten, ferro-vanadium, ferro-uranium, ferro-molybdenum, ferro-nickel or metallic nickel and ferro-cobalt or cobalt metal, are added to the steel, in the molten state in the furnace, or after 20 it is tapped in the ladle. As the regular commercial grades of such ferro-alloys contain an appreciable amount of carbon, this practice introduces an undue amount of carbon in the steel. If special grades of low-carbon-ferro-alloys are used, the cost of such alloys is comparatively so high as to prohibitively increase the cost of steel produced. These defects are especially apparent in the 25 case of steels where the content of the alloying element has to be high and the carbon content low, as in the case of the so-called "stainless" steels or irons, which have a chromium content of between 9 and 15% and a low carbon content.

It is not commercially practicable to use the regular high carbon ferro-alloys, and then decarbonize the steel after their addition, as the process of oxidizing the carbon is accompanied by an oxidation, and consequent waste, of the valuable alloying elements.

Another deficiency of the existing methods of manufacturing alloy steels, by the addition of metallic ferro-alloys to 45 molten steel, is the phenomenon of segregation. The alloy being added in the solid state in the form of lumps scattered over the surface of the molten steel, causes points of concentration of the alloying element at the 50 location of each of the lumps. As the steel is tapped immediately after melting of the lumps in order to avoid an undue oxidation of the alloying element, these points of higher concentration have no opportunity 55 to equalize themselves over the entire mass of metal by diffusion. Moreover, the ferro-

alloys have various constituents of different melting points and degrees of solubility, as for example the carbides in the ordinary grades of alloy. Such carbides have a 60 higher melting point than the remainder of the alloy. Such a carbide-containing ferro-alloy, when added to molten steel, will have the result that when the rest of the alloy will be completely assimilated, the carbide 65 content will still be in the solid state, floating in the molten steel, without giving up its alloying element content to the bath. Such solid particles with a high alloying element content will persist in the steel on 70 solidification and present segregation.

I overcome the above mentioned difficulties by introducing the alloying metal in unreduced form, such as an oxide or an ore, and reducing it simultaneously with the 75 melting of the cold metal, such as the steel scrap to be melted. The alloying metal ore or the scrap and the reducing agent may all be charged cold into the furnace, preferably mixed together, and then melted. On the 80 other hand, a molten bath containing a part of the iron and steel, together with the reducing agent if desired, may be formed, and then the cold scrap and alloying ore, with or without a reducing agent, may be 85 charged into the furnace. In either case, the alloying ore is reduced simultaneously with the melting of some or all of the iron or steel. In each case the unmelted metal, such as steel scrap, is a substantial quantity 90 or proportion of the whole charge melted, so that the dissemination of the alloying metal into the steel which is being melted simultaneously with the reduction of the alloying metal, results in a substantially 95 thorough dissemination throughout the body of the charge. The freshly reduced alloying metal is in direct contact with the melting steel, and therefore the best conditions are obtained for the alloying and uniform 100 disseminating of the alloying metal throughout the molten steel. The alloying element is obtained from a cheap source. The introduction of carbon and segregation are avoided in the finished steel.

The action of the alloying oxide or ore in oxidizing the reducing agent and the action of added fluxing material, generally lime, in absorbing and neutralizing the 110 oxidized reducing agent together with undesirable metalloids, such as phosphorus and sulphur, cause a refining of the steel to take

place simultaneously with the production of the alloy and melting of the scrap.

The process may be carried out in the following manner:

- 5 The steel or iron scrap desired to be melted to the alloy steel preferably selected in comparatively small sizes, such as borings, turnings, etc., is mixed with a reducing agent, which may be a metallic reducing agent such as silicon, manganese, calcium magnesium or the like, either alone or in combination with a carbonaceous reducing material, for instance, a carbide such as pig iron or wash metal. To this mixture is added the alloying 10 raw material, such, for example, as chromite, preferably in the presence of lime or lime, fluorspar and borax, as a flux. The quantity of reducing agent and alloying raw material are figured such as to give the requisite percentage of alloying element in the total weight of finished steel. The purpose and function of the flux is to produce a slag with the gangue of the raw material containing the alloying element, and is of such a nature 15 as to effectively remove by chemical combination the product formed by oxidation of a metallic reducing agent, such as silicon. In the case of silicon, the silica produced by its oxidation goes into chemical combination 20 with the slag, principally in the form of calcium silicate, and is thereby removed from the metal. The practical result achieved by the flux, therefore, is the prevention of the presence of the reducing agent in the finished steel. The flux also combines with the refractory gangue elements of ore and renders the oxide more amenable to reduction 25 by the reducing agent. The reducing reaction then proceeds at the same time the scrap is melted and the reduced alloying element is directly in contact with the melting scrap and is readily absorbed in the liquid steel. As this operation takes place in the presence 30 of the fluxing materials, a refining of the molten scrap proceeds simultaneously. The mixture of raw materials as above described is charged into any well known steel making furnace such as an open-hearth, or crucible, or electric furnace at a temperature suitable 35 for the reaction. After the reaction is complete and the entire charge thoroughly molten, it is advantageous to raise the furnace temperature in order to eliminate the last traces of the reducing agent in the finished 40 steel, accelerating the effect produced by fluxing agents added for this purpose.

The process is particularly applicable to the manufacture of alloy steel or iron in an electric furnace. The furnace may be operated continuously, the steel or iron being tapped out as collected, and the unmelted scrap or pig, the alloying ore, the reducing agent and the slag-forming flux may be charged continuously or at short intervals to the bath, which is continuously maintained

on the hearth. This allows an electric furnace to be operated continuously at substantially constant load, thus obviating the power fluctuations incident to periodic operation of an electric smelting furnace.

The most generally adapted metallic reducing agent is ferro-silicon. However, silicon metal or any other silicon alloy such as a silicon alloy containing one of the alloying metals may also be advantageously used. For instance, in the case of the manufacture of so-called "stainless" steel, a silico-chromium alloy may be added to the raw cold charge and its silicon content utilized to reduce a further quantity of chromium from chrome ore present in the charge. This procedure is especially advantageous in the case of a steel containing a high percentage of the alloying element.

The term "silicon reducing agent" is intended as a term of general description and not of limitation, and is intended to include not only substantially pure silicon, but also silicon alloyed with other metals or metalloids.

In the case of alloy steels containing a plurality of alloying elements, this procedure may be carried out in the same manner, the raw materials in the right proportions containing the plural elements, being charged together with the scrap and reducing agent. The flux may be added separately or the raw alloying materials may be selected of such a composition as to have in their gangue the necessary fluxing components.

The steel scrap and the ore may be mixed together and the mixture charged into the furnace or the steel scrap and the ore may be introduced in separate batches or charges, so long as they are charged substantially simultaneously or within such time interval that the melting down of the scrap will proceed substantially simultaneously with the reduction of the ore.

Also a plurality of reducing agents may be used, such as a mixture of carbonaceous and metallic reducing agents or several different metallic reducing agents. For instance, a ferro-silicon alloy containing carbon may be used, both its silicon and carbon contents being utilized for the reduction purpose. Also any reducing agents originally present in the scrap may be effectively used, thus eliminating their presence from the finished steel. Also the fluxes added to the charge will have the effect of refining the molten scrap of its metalloid contents, such as sulphur and phosphorus, simultaneously with the melting of the scrap and its alloying with the alloying element.

If desired, after the melting of the charge is complete and the reaction is ended, a small quantity of additional ferro-silicon or ferro-manganese may be added as a deoxidizing agent.

cleanser, before tapping the steel, as is the common practice in making alloy steels.

The advantages of this process of simultaneous melting, refining and alloying are especially marked in the case of using silicon as a reducing agent, and producing steels or iron with a high alloy content and very low carbon content. As such an instance may be cited the manufacture of so-called "stainless" iron containing 9 to 15% chromium and less than 0.1% carbon. Also the advantages of this process are apparent in the case of alloying a highly oxidizable and difficultly soluble element as uranium in steel. The alloying element being produced in the nascent state and directly in contact with the melting steel, the chances of its oxidizing or not dissolving are reduced to a minimum. Also, as the carbon content of the finished steel can be eliminated to any desired extent, simultaneously during the process of reducing and alloying, the exact percentage of carbon in the finished alloy steel can be arrived at more accurately by recarburizing before tapping. In the case of metallic reducing agents being used, their presence in the finished steel is practically eliminated by the action of fluxes. Thus by the process of this invention a steel of predetermined given composition can be more accurately produced than by the use of ferro-alloys. Also by this process, as the valuable alloying elements do not exist at any time in the metallic state, unless dissolved and alloyed in the steel itself, and as after their solution in the steel there is no occasion to subject such steel to an oxidizing process for removal of carbon, for instance, as in the older processes, there is no loss suffered through oxidation, rendering the process extremely economical.

The charge put into the furnace contains a sufficient proportion of steel scrap so that the metal as tapped from the furnace is a finished steel, as contrasted with a cast iron or a ferro-alloy. The term "steel", however, as herein employed, is intended as a term of general definition and not of limitation, and is intended to include steels having very low carbon and metalloid contents and which are sometimes called "irons", as for example, the so-called "stainless irons".

The process also assures a thorough and uniform dissemination of the alloying metal throughout the body of the molten iron or steel before tapping.

While the preferred method of carrying out my process has been specifically described, it is to be understood that the invention is not limited to all of the described details, but may be otherwise embodied in processes of making alloy steels or irons, within the scope of the following claims.

I claim:

1. The process of making chrome steel, comprising maintaining a molten bath of chrome steel in the furnace, tapping the steel therefrom from time to time, and charging into the bath as required a silicon reducing agent and a metalloid-absorbing lime-containing flux material and steel scrap and an unreduced chromium compound in amounts sufficient to furnish the major portion, if not all, of the iron and chromium contents of the steel and proportioned to maintain the desired composition of the steel bath, substantially as described.

2. The process of making alloy steel, comprising maintaining a molten bath of alloy steel in a furnace, tapping the steel therefrom from time to time, and charging into the bath as required a metallic reducing agent and a metalloid-absorbing lime-containing flux material and steel scrap and an unreduced compound of the alloying metal in amounts sufficient to furnish the major portion, if not all, of the iron and alloying metal contents of the steel and proportioned to maintain the desired composition of the steel, substantially as described.

3. The process of making chrome steel, comprising maintaining a molten bath of chrome steel in a furnace, and charging into the bath as required a silicon reducing agent and steel scrap and an unreduced chromium compound in amounts sufficient to furnish the major portion, if not all, of the iron and chromium contents of the steel and proportioned to maintain the desired composition of the steel bath, substantially as described.

4. The process of making chrome steel, comprising forming a charge containing a silicon reducing agent and steel scrap and an unreduced chromium compound in amounts sufficient to furnish the major portion, if not all, of the iron and chromium contents of the steel, and simultaneously melting the charge and reducing the chromium from its unreduced compound, substantially as described.

5. The process of making chrome steel, comprising forming a charge containing a silicon reducing agent and a metalloid-absorbing lime-containing flux material and steel scrap and an unreduced chromium compound in amounts sufficient to furnish the major portion, if not all, of the iron and chromium contents of the steel, and simultaneously melting the charge, reducing the chromium from its unreduced compound and refining the steel, substantially as described.

In testimony whereof I have hereunto set my hand.

BY RAMJI D. SAKLATWALLA.